

# UNITED STATES PATENT OFFICE.

QUIRINO SESTINI AND TITO RONDELLI, OF BERGAMO, ITALY.

## BRONZING OR COLORING OF METALLIC SURFACES.

1,277,761.

Specification of Letters Patent. Patented Sept. 3, 1918.

No Drawing.

Application filed May 15, 1917. Serial No. 168,763.

*To all whom it may concern:*  
Be it known that we, QUIRINO SESTINI and TITO RONDELLI, subjects of the King of Italy, residing at Bergamo, Italy, have invented certain new and useful Improvements in or Relating to the Bronzing or Coloring of Metallic Surfaces, of which the following is a specification.

This invention relates to "bronzing" or 10 coloring metallic surfaces, its object being to provide, among other things, a process whereby metallic surfaces can be "bronzed" or colored both rapidly and with a finish that is adherent, durable and fine. Further 15 it affords a choice in the kind of color produced on the surface.

The term "bronzing" is employed throughout this specification and in the claims to denote not merely the production of the coloration known as "bronzing" but the formation of a coating of an oxid of copper or of iron which serves as a protection to the surface beneath it to prevent further oxidation or corrosion thereof. Prominent among the 25 objects of the present invention is the provision of a process whereby the desired results can be obtained more rapidly than hitherto. To this end the surface to be protected or colored is preliminarily coated 30 with an electrolytic deposit of iron or copper.

According to the present invention a surface is "bronzed" or colored by depositing copper or iron electrolytically thereon and 35 subsequently "oxidizing" the said deposited metal; by "oxidizing" is meant not merely the production of a simple oxid but the production of any compound obtained by a process which in the broadest chemical sense 40 may be described as an "oxidizing" process.

The bath employed according to this invention is preferably a hot dense alkaline solution containing an oxid either of copper or of iron combined with an oxid of the alkaline metal present; and the "bronzing" or 45 coloring is conveniently effected by first electrolytically depositing the iron or copper on the surface to be treated in a bath of the kind just stated and subsequently coloring 50 the said deposit by reversing the current.

The density of the solution varies between about 1.25 and 1.55 and the temperature at which it is worked is from about 115° C. upward, the term "density" being used in this

instance, as in all others herein, to indicate 55 the specific weight of the solution as compared with that of water.

The process may be carried out by making the conducting surface anode, or alternately cathode and anode, but finally anode 60 in an electrolyte that is a hot dense alkaline solution such as has been above referred to and that contains an oxid either of copper or of iron combined with an oxid of the alkaline metal present, the said combined substance being either a ferrite of the alkali metal, or a similar copper compound thereof. The temperature of the bath is conveniently between about 120° C. and 140° C. and its density between 1.3 and 1.5 due to the 70 alkaline content.

In order to provide a bath for the purposes of the present invention, the bath may be prepared, as part of the present invention, by repeatedly reversing the current 75 through a hot dense alkaline solution between electrodes that are both of iron or both of copper; the alkaline solution may be either a caustic alkali or an alkaline carbonate and have a density between 1.3 and 80 1.4 and a temperature between about 120° C. and 130° C.

A further step provided by the present invention, to be used as and when desired, consists in immersing the surface that is being treated, after it has been electrolytically colored in a solution of caustic alkali containing between about 10% and 20% of a metallic nitrate, or an aromatic nitrate derivative as nitrophenols or nitronaphthols; 90 the density of the solution should be about 1.4 and its temperature about 140° C.

All or any of the above described steps may be followed by drying the colored surface and leaving it long immersed in a bath 95 of oil at a temperature of between about 150° C. and 180° C.; the period of immersion may be in the neighborhood of about ten minutes and the oil employed is conveniently olive oil, or a mixture of linseed or 100 mineral oils.

The following examples serve further to disclose the present invention:

An electrolyte is prepared by passing current and repeatedly reversing it between 105 electrodes of the metal to be used, namely either iron or copper in a bath of hot concentrated alkali. The density of the bath,

for a caustic alkali, is between 1.3 and 1.4; equivalent quantities of caustic potash or an alkaline carbonate may equally be used.

The temperature of the bath is raised to 5 a point between about 120° C. and 130° C. If the electrodes are of wrought or cast-iron, or of steel, the repeated reversals of current through it causes an oxid of iron to be formed and dissolved in or to be combined with the alkali in the bath; apparently the result is the formation of an alkaline ferrite having the formula  $Fe_2O_3 \cdot Na_2O$  or  $NaFeO_2$ .

If the electrodes are of copper it is an 15 oxid of copper which is formed and enters into the electrolyte and forms a solution of a compound whose formula is similar to that of the iron compound above referred to but with copper as its metallic element.

20 When once the electrolyte has thus been prepared it may be used indefinitely and does not undergo exhaustion.

Assuming iron electrodes to have been used so that the electrolyte contains an iron 25 oxid and the article to be colored is to be colored a bright black, it is immersed in the bath, the bath is brought to a temperature of about 120° C. to 130° C. and the article is made to act as cathode for about 1 to 2 30 minutes. The article does not need to be preliminarily cleaned but may be immersed whether smooth or rusty direct in the bath. The current density employed is about 5 amperes per square decimeter of the 35 surface to be colored.

While thus operating as cathode the article is both cleaned and plated with electrolytic iron. At the end of this period the current is reversed and the article made to 40 serve as anode for from six to eight minutes.

The result of this step is to form a bright 45 black coating of oxid upon the article which may, however, be further strengthened and rendered more adhesive by subsequently immersing it for a few minutes in a solution of caustic soda having a density of 1.4, heated to about 140° C. and containing from 10% to 50% of sodium nitrate. Instead of sodium nitrate almost any metallic nitrate or aromatic nitro derivative may be employed in this solution.

If a dull black is desired the current should be reversed at least two or three 55 times, taking care, however, to make the final direction such that the article acts as anode and that the current is continued for at least two minutes after the oxidation is complete. The completion of the oxidizing action is indicated by the voltage at the 60 terminals of the bath; during the oxidizing process the voltage is in the neighborhood of 0.6 volts but rises to between 1.8 and 2 volts when oxidation is complete.

The colored articles, whether bright or 65 dull, are dried and immersed for ten minutes

in a bath of olive oil heated to between 150° C. and 180° C. Instead of olive oil a mixture of linseed oil and mineral oil may be employed. Brushing the colored surface causes it to become brighter and brighter.

If red or yellow shades of coloration are desired, the concentration of the bath must be increased to about 1.5 and the temperature to about 140° C. Nitrate of soda or other oxidizing agents may also be added.

When arrangements have been made to deal with articles by a regular routine the complete treatment of each batch takes from ten to fifteen minutes so that a batch is fully treated in approximately that time.

If it is desired to use a copper surface and color it the above processes described with reference to iron may be employed, using, however, copper electrodes and employing the conditions of temperature and concentration of the electrolyte given above for the black coloration of iron. The coloration is understood to be due to the formation of a closely adhering layer of oxid of iron or of copper as the case may be on the 90 surface of the anode.

In a modified form of the process, the surface to be colored is covered with a deposit of electrolytic iron or copper which is subsequently oxidized by a simple immersion 95 in an alkaline oxidizing solution, such as a solution of nitrate of sodium or other metallic nitrate, or aromatic nitro derivative.

The process, according to this invention, is easy to carry out and economical; the consumption of energy does not ordinarily exceed one watt hour per square decimeter of the surface treated. The consumption of the electrolyte is so slight as to be negligible. The heating of the bath may be carried out 105 in any desired manner, but preferably by means of gas or electricity.

Having now particularly described and ascertained the nature of our said invention, and in what manner the same is to be performed, we declare that what we claim is:

1. The herein-described process of electrolytically coloring metallic surfaces, which consists in temporarily inserting the object to be treated, as a cathode, in a hot, 115 dense alkaline solution containing an oxid of the metal to be deposited combined with an oxid of the alkali metal present; passing current through the electrolytic bath to deposit on the surface of said object a film of the first-mentioned metal; and exposing the surface so treated to oxidizing conditions in an alkaline bath.

2. The herein-described process of electrolytically coloring metallic surfaces, which 125 consists in temporarily inserting the object to be treated, as a cathode, in a hot, dense alkaline solution containing an oxid of the metal to be deposited combined with an oxid of the alkali metal present; passing current 130

through the electrolytic bath to deposit on the surface of said object a film of the first-mentioned metal; and temporarily reversing the passage of the current through the bath 5 and inserting the said object therein as an anode, so as to set up an oxidizing condition in the said bath for action on the surface so treated.

3. The herein-described process of electrolytically coloring metallic surfaces, which 10 consists in temporarily inserting the object to be treated, as a cathode, in a hot, dense alkaline solution containing an oxid of the metal to be deposited combined with an oxid 15 of the alkali metal present; passing current through the electrolytic bath to deposit on the surface of said object a film of the first-mentioned metal and oxidizing the surface so treated in an alkaline bath containing an 20 oxidizing compound.

4. The herein-described process of electrolytically coloring metallic surfaces, which 25 consists in temporarily inserting the object to be treated, as a cathode, in a hot, dense alkaline solution containing an oxid of the metal to be deposited combined with an

oxid of the alkali metal present and an alkaline nitrate; passing current through the electrolytic bath to deposit on the surface of said object a film of the first-mentioned metal and exposing the surface so treated to oxidizing conditions in an alkaline bath. 36

5. The herein-described process of electrolytically coloring metallic surfaces, 35 which consists in passing current and repeatedly reversing it between electrodes of the metal to be deposited in a bath of hot concentrated alkali to form an electrolyte comprising an oxid of the first-named metal 40 combined with an oxid of the alkali metal present; temporarily inserting the object to be treated, as a cathode, in said electrolytic bath to deposit a film of said first named metal on the surface of said object; and exposing the surface so treated to oxidizing 45 conditions in an alkaline bath.

In testimony whereof we affix our signatures.

PROF. QUIRINO SESTINI.  
DR. TITO RONDELLI.